

## UNITED STATES PATENT OFFICE.

MORTON SULTZER, OF BROOKLYN, NEW YORK, ASSIGNOR TO WESTERN ELECTRIC COMPANY, INCORPORATED, OF NEW YORK, N. Y., A CORPORATION OF NEW YORK.

## METHOD OF COATING CONDENSERS.

1,210,722.

Specification of Letters Patent.

Patented Jan. 2, 1917.

No Drawing.

Application filed June 24, 1916. Serial No. 105,681.

*To all whom it may concern:*

Be it known that I, MORTON SULTZER, a citizen of the United States, residing at Brooklyn, in the county of Kings and State of New York, have invented certain new and useful Improvements in Methods of Coating Condensers, of which the following is a full, clear, concise, and exact description.

10 This invention relates to a method of coating condensers in order to prevent the admission of moisture and to enable them to withstand rough usage and large variations in temperature.

15 Standard condensers are usually manufactured of alternate plates of tin foil and mica impregnated with a wax, usually paraffin. In order to protect the finished units from the admission of moisture, they are usually dipped in paraffin or some such wax. When, however, such condensers are used in telephone circuits and are exposed to the elements, it has been found that at low temperatures, such as 10 degrees Fahrenheit, 20 the coating of paraffin will crack and fall off, leaving the unit unprotected. It is desirable, therefore, to supply a condenser with a more substantial coating, particularly one which is more impervious to moisture than paraffin, and one which will withstand climatic variations of temperature.

25 The difficulty, however, with coating such condensers as described above with a more rugged coating is due to the fact that, if the condenser unit is raised to a temperature of 120 degrees Fahrenheit or more, it takes a permanent set and its calibration is thereby destroyed. This results from the fact that the melting point of paraffin is in the 30 neighborhood of 120 degrees Fahrenheit.

40 A compound which has been used extensively for coating and sealing electrical apparatus such as condensers must be raised to a temperature of about 300 or 350 degrees 45 Fahrenheit. As an illustration of the difficulties encountered in coating standard condensers with such a compound, it may be stated that a condenser of the above description was dipped in such a molten compound, and it was found that the capacity of the unit had changed about four per cent.

50 In this invention, I have devised a method of treatment whereby a coating of such a compound with a high melting point may be applied to electrical apparatus impregnated

with such a material as paraffin without seriously affecting the calibration of the apparatus and the method consists essentially in placing such apparatus impregnated with a compound of a low melting point in particular, mica condensers, in a desiccator to remove all traces of moisture. The desiccator is then placed in a refrigerator and is cooled to a low temperature in an atmosphere of dry air. Immediately 60 upon being removed, the condensers or other apparatus are dipped into a high melting point compound and immediately withdrawn. In this way, the temperature of the unit itself is never raised to a point where 65 the impregnation may be softened, which softening would result in a change of capacity or other electrical dimensions.

70 Although I do not wish to be limited as to the extent of precooling, I have found 75 that with condensers impregnated with paraffin, and which are to be dipped into some suitable compound having a melting point ranging from 300 to 350 degrees, that it is generally sufficient to precool the 80 condensers to a temperature of approximately 10 degrees Fahrenheit.

85 While this invention has been described specifically in connection with mica condensers, it is apparent that the method of precooling and dipping is equally applicable to any form of condensers, such as paper condensers, and that it is also applicable to apparatus other than condensers, such as inductance coils, transformer windings etc., 90 where the conditions to be met with are substantially the same.

95 What is claimed is:

1. The method of coating with a high melting point compound, electrical apparatus containing a low, melting point compound, which consists in precooling the apparatus and dipping it in and quickly removing it from the molten compound of high melting point.

100 2. The method of coating with a high melting point compound, electrical apparatus containing a low melting point compound, which consists in precooling the apparatus and dipping it in and so quickly removing it from the molten compound that the low melting point compound is not permanently affected.

105 3. The method of coating with a high melting point compound, a condenser im-

pregnated with a low melting point compound, which consists in precooling the apparatus and dipping it in and so quickly removing it from the molten compound that the low melting point compound is not permanently affected.

4. The method of coating with a high melting point compound, a condenser im-

pregnated with paraffin, which consists in precooling the condenser and dipping it in 10 and so quickly removing it from the high melting point compound that the paraffin is not raised to a dangerous temperature.

In witness whereof, I hereunto subscribe my name this 23rd day of June, A. D. 1916. 15

MORTON SULTZER.

**Copies of this patent may be obtained for five cents each, by addressing the "Commissioner of Patents, Washington, D. C."**